

April 11, 1944.

G. S. HOOPER

2,346,258

METHOD FOR PRODUCTION OF CELLULOSE ACETATE STAPLES

Filed June 13, 1941

Fig. 1.



Fig. 2.



INVENTOR.

Gilman Stanley Hooper

BY

*A. Nathan Snyder*

ATTORNEY.

## UNITED STATES PATENT OFFICE

2,346,258

METHOD FOR PRODUCTION OF CELLULOSE  
ACETATE STAPLEGilman Stanley Hooper, Waynesboro, Va., assign-  
or to E. I. du Pont de Nemours & Company,  
Wilmington, Del., a corporation of Delaware

Application June 13, 1941, Serial No. 397,990

1 Claim. (Cl. 18—47.5)

This invention relates to the production of cellulose acetate staple. More particularly, the invention is directed to the crinkling of a very large bundle of continuous filaments and the cutting of this crinkled bundle to produce staple of substantially uniform length, of good strength, with a desirable crinkle and well-opened.

In order to satisfactorily spin rayon staple it is highly desirable that the staple have a retentive crimp. It is also desirable that the crinkled staple fiber should have substantially the original strength of the filament, and that the bundle of staple should be uniformly open, i. e., it should be fluffy and free of stuck or coalesced fibers. In the manufacture of cellulose acetate staple no satisfactory method has heretofore been devised which achieves all of these desiderata.

It is, therefore, an object of this invention to provide an improved process for the production of crinkled cellulose acetate staple which is eminently suited for the production of spun yarn. Another object of this invention is to provide optimum conditions of crinkling so that the number of crimps per inch and the intensity of crimp can be controlled satisfactorily without substantially impairing the strength of the filaments. Still another object of this invention is to provide optimum conditions for cutting the bundle of crinkled filaments so that substantially all the crinkle is retained in the cut fibers, so that substantially uniform fiber lengths are produced, and so that the cut fibers fly apart or explode to give an exceedingly well-opened and fluffy product. A still further object is to provide a novel tow of crinkled filaments which is admirably suited for direct conversion into a top. Other objects will be apparent from the description that follows.

These objects are accomplished by my invention which, briefly stated, comprises imparting, by purely mechanical means, a crinkle of predetermined frequency and amplitude to a tow of continuous filaments of cellulose acetate, the solvent plus moisture content of which is adjusted and maintained during the crinkling operation within limits hereinafter specified. Thereafter the crinkled tow is converted to staple by cutting the same in air with a sharp knife or other cutting device, while maintaining the tow under a slight but positive tension, and while further maintaining the solvent plus moisture content of the tow within a range to be hereinafter specified. The resulting crinkled staple is subsequently treated to bring its solvent content to less than 1.5% and to adjust its moisture content to about

6.5% based on the weight of the dry fibers. After this, the staple fibers may be sprayed with a liquid containing an anti-static agent, blended by a mechanical blender, and packaged.

Tow, mechanically crinkled under the conditions of this invention, and comprised of cellulose acetate filaments within the range of 3 to 20 denier, and preferably within the range of 5 to 12 denier, containing from 6 to 12 crinkles per inch, the crinkles ranging in amplitude from  $\frac{1}{8}$  to  $\frac{1}{4}$  inch, is especially suited for use in cutting and drawing apparatus designed for the direct conversion of tow to top. As a practical matter, however, plants equipped for the preparation of tow are not equipped for the direct conversion of tow to top; hence, for this purpose, the tow must be packaged and shipped to the point where it is to be cut and drawn and eventually spun into yarn. Tow containing the high percentage of solvent plus moisture required in the crinkling operation cannot be wound into packages and stored for any length of time without seriously reducing the essential intensity and uniformity of the crinkle. Therefore where tow, crinkled according to my process, is to be employed in tow-to-top converters, it is prepared for shipment by treating the same in relaxed condition to remove substantially all of the solvent and to adjust the moisture content to about 6%, after which it is wound into suitable packages. Crinkled tow thus conditioned and meeting the specifications above recited, is a further feature of my invention.

The preferred mode of imparting crinkle to the tow of cellulose acetate is to mechanically pleat or put serrations in the tow generally transversely of the longitudinal axis thereof, in apparatus of the type described in U. S. patent application Serial Number 368,925, filed Dec. 6, 1940, by Ira V. Hitt, now U. S. Patent No. 2,311,174, wherein the tow is passed between two positively driven, smooth-surfaced rolls, and into a relatively small chamber where it is momentarily piled or jammed in folds between a yieldable clapper plate and the bite of the rolls. The individual filaments of the tow issuing from this apparatus are uniformly crimped and the tow is substantially free of stuck or fused filaments.

As previously indicated, it is essential that the moisture plus solvent content of the filaments be maintained within certain limits to get optimum results at the crinkler, and at the cutter where the crinkled tow is directly converted to staple. The moisture plus solvent content of the filament bundle depends upon the denier of

the filaments and the limits for satisfactory operation can best be expressed by the following formulae. To secure satisfactory crinkling of bundles of cellulose acetate filaments, the moisture plus solvent content should be satisfied by the following formula wherein  $d$ =denier of the filament:

Per cent moisture+solvent=40×log  $d$ — $d$ +2±6  
but in no case should the moisture plus solvent content be greater than 40% or less than 8% based on the dry weight of the cellulose acetate filaments.

At the cutter, the moisture plus solvent content should be satisfied by the formula:

Per cent moisture+solvent=40 log  $d$ — $d$ ±6  
but in no case should the amount of solvent plus moisture be greater than 38% or less than 5% based on the dry weight of the filaments.

The ratio of moisture to solvent is not extremely important but, in general, the ratio is much higher for low deniers than for heavy denier filaments. For instance, in crinkling, the solvent may comprise as little as 15 to 20% of the total moisture plus solvent present in 1.5 denier filaments but the solvent content may be as high as 70% or more in the case of heavy denier filaments such as 20 denier. The same is generally also true for the moisture-solvent content of the filaments at the time of cutting.

Another critical element to enable satisfactorily opened staple to be produced at the cutter is the necessity of keeping the rope as it is being cut in the air with a single sharp knife edge under a predetermined, low tension. Even if the crinkled rope contains the optimum solvent-moisture content, if cut when held under substantially no tension it will not explode or fly apart as is desired and if the tension is too great, the crinkle will be removed and hence the desired crinkle in the cut staple will not be present. Tensions between 0.005 and 0.04 gram per denier are essential to obtain good opening of the staple and, at the same time, maintain the crinkle in the cut fibers.

The essential operations involved in the conversion of a tow of continuous filaments of cellulose acetate to crinkled staple suitable for the production of spun yarn, according to my invention, will now be described in connection with the accompanying drawing wherein:

Fig. 1 is a diagrammatic illustration of the operations for forming a tow and crinkling the same, and

Fig. 2 illustrates diagrammatically the conversion of the crinkled tow to staple.

Referring to Fig. 1, cellulose acetate yarn formed by the dry or evaporated method is drawn from spinning cell 1 by feed roll 2, and thence over guide 3 after which it is combined with yarns being simultaneously produced in similar units to form a tow which is preferably from 30,000 to 50,000 denier in size. If desired, any suitable finish composition may be applied, and preferably at a point intermediate draw roll 2 and guide 3, by any suitable means (not shown) such as applicator rolls, fountain sprays, wicks, and the like. Where it is necessary to reduce the moisture plus solvent content of the tow in order to bring it within the optimum conditions above defined, the tow may be subjected to moderate drying, e. g., by passing the same through a drier 4. The combined yarns forming the tow, now properly conditioned, are fed over a guide

5 roll 5 and into a crinkler 6 of the type disclosed in U. S. patent application Serial No. 368,925 (Hitt). The crinkled tow is collected in a can 7 eccentrically mounted on a revolving platform 8. To form staple, the crinkled tow is passed over guide roll 9, is preferably combined with like tow from other containers and the combined tow is fed through feed rolls 10 and 11 and into a centrifugal cutter 12, where it is cut in air under moderate tension. The well opened staple, thus produced, is collected in hopper 13 or in any other suitable container, after which it may be immediately spun or, if desired, conditioned for storage and shipment.

15 The following examples further illustrate the invention.

#### EXAMPLE I

##### (Three denier per filament staple)

20 450 denier, 150 filament cellulose acetate yarn was spun by the dry or evaporative method from an acetone solution and was drawn from the cell with a solvent content of approximately 15%. Ten per cent of an aqueous emulsion of oils, such as are commonly used in the finishing of textile fibers, was applied to the bundle of continuous filaments immediately after emersion from the spinning cell. Filament bundles from a number of cells were then collected into a very heavy denier bundle or tow, for instance having a total denier of approximately 28,000 (approximately 9,300 filaments) and this tow was fed into the crinkler described in U. S. patent application Serial No. 368,925 (Hitt) at the rate of 220 yards per minute. During the passage from the spinning cell to the crinkler, the tow was subjected to a certain amount of drying which brought the total moisture plus solvent content of the tow at the crinkler down to about 19%, consisting of 25 approximately 7% solvent and 12% moisture. (The moisture being moisture applied as a finish emulsion and moisture originally contained in the spinning solution.) The crinkler was adjusted so that approximately 12 crinkles per inch of  $\frac{1}{16}$  inch amplitude were inserted in the continuous filaments comprising the bundle. The bundle of crinkled filaments leaving the crinkler was collected in a solid fiber barrel and stored without drying until ready for cutting. As spun, the yarn had a dry strength of 1.40 grams per denier and 28% elongation. After crinkling, the dry strength was 1.28 grams per denier with approximately the same elongation, whereas in the absence of control of moisture plus solvent, the dry strength of crinkled filaments would frequently fall to 0.7 gram per denier which made the product unsatisfactory.

25 The tows of crinkled continuous filaments were cut in a centrifugal type cutter having a single stationary cutting blade such as described in U. S. Patent No. 1,723,998 (Beria). The moisture plus solvent content of the tow was allowed to decrease through storing so that as it was fed to the cutter, it contained about 14% of which about 4% was solvent. Four tows were combined and fed to the cutter at the rate of 200 yards per minute and by rotating the cutter disc at 3600 R. P. M. A tension of approximately 0.1 gram per filament was applied to the filament bundle and well-opened, fluffy, wool-like fibers of 2 inches in length were produced. The crinkled staple collected from the cutter was fed by suction to a feed hopper of a continuous drying apparatus wherein the solvent content was reduced to below 1.5% and the moisture adjusted to 6.5%

based on the dry weight of the fibers. On leaving the drier, the staple fibers were conveyed by air to the feed hopper of an opening device where 0.1% cetyl betaine was sprayed on the fibers to inhibit build-up of electrostatic charges thereon in subsequent operations. The fibers are then passed through a blender consisting essentially of a pin type beater and carried by air to a receiving bin, from where the staple could be dropped into a baler.

EXAMPLE II

(Twelve denier per filament staple fiber)

Cellulose acetate yarn of 12 denier per filament (816 denier, 68 filaments) was drawn from the dry spinning cell and approximately 8% of an aqueous emulsion of finishing agents was applied thereto to facilitate subsequent processing. The filament bundles from several cells were collected together to form a tow of about 50,000 denier and, after a mild drying action, was fed through the crinkler described in the Hitt application at the rate of 123 yards per minute. The moisture plus solvent content of the tow at the crinkler was approximately 30% of which 22% was solvent (acetone). Approximately eight crinkles per inch of  $\frac{1}{8}$  inch amplitude were inserted in the filaments as they passed through the crinkler. The tow of crinkled filaments leaving the machine was collected in solid fiber barrels and stored for cutting. Tensile tests on the crinkled and uncrinkled filaments showed that about 80% of the original strength had been retained through the crinkling operation.

Three of the crinkled tows so produced were subsequently brought together and passed into a centrifugal type cutter such as previously referred to, at the rate of 250 yards per minute and with the centrifugal disc revolving at 1800 R. P. M., the average tension on each filament at the time of cutting was in the neighborhood of 0.20 gram, and the length of the staple produced was 5 inches. The moisture plus solvent content of the tow at the cutter was 26%, of which 19% was solvent. The cut fibers flew apart at the cutter in the same manner as described in the previous example to produce a well-opened product which was passed continuously to the hopper of the drier; dried to 1.5% or less solvent content and 6.5% moisture content; sprayed with an anti-static finish consisting of 0.4% of lorolamine hydrochloride on the weight of the fibers; and then passed directly to a storage bin without any additional opening action. The fibers produced in this manner were baled and sold for use in the worsted industry.

The invention is not of course limited to the exact conditions and manipulations set out in the above examples, but is susceptible rather to wide variation and modification, observing at all times, however, the several critical factors hereinbefore recited, and the following generalities.

The optimum moisture plus solvent content of the rope at the crinkler and cutter varies as a function of the denier of the material being handled. For example, fine denier filaments such as 1.5 should contain relatively little moisture and solvent when crinkled and when cut. The use of higher amounts of moisture and solvent will result in extremely intense crinkles and very serious weakening of the filaments in the crinkling operation, and if cut while they contain too high a concentration of moisture plus solvent, the filaments will not spring apart, but will give a mass of essentially unopened fibers. As the filament

deniers increase, however, not only can higher moisture plus solvent contents be tolerated, but such higher moisture plus solvent contents are necessary if satisfactory crinkling and cutting are to result. If the moisture plus solvent content of heavy denier filaments is maintained at too low a level, the material may be incapable of being crinkled or, at best, the crinkle will be large, non-uniform, and lacking in permanence, and of little value as an aid in subsequent processing of the staple fiber into spun yarn. Also in cutting, filaments of higher deniers have a greater tendency to spring apart than small denier filaments and, for this reason, higher moisture plus solvent contents can be tolerated and are necessary in order to maintain the filament in a suitable pliable condition.

Not only is the moisture plus solvent content of the tow essential for the production of uniform length, well-opened, fluffy fibers, but it is also essential that the tension on the tow at the time of cutting be maintained within definite limits. To get uniform lengths of cut staple, it has been found desirable to tension the tow slightly at the feed rolls before it enters the cutter disc. If the moisture plus solvent content of the tow is too great, a portion of the crinkle may be removed from the filaments at this point. Accordingly, control of moisture plus solvent and control of tension are both essential to maintain the desirable amount of crimp in the staple product and to obtain a well-opened and uniform length product.

The excellence of individual fiber crinkles is of outstanding importance and enables large denier fibers to be readily formed in spun yarns without necessitating special apparatus. By suitable adjustment, the frequency and intensity of crinkle may be varied through a wide range, say from 5 to 30 crinkles per inch with amplitudes of from  $\frac{1}{64}$  of an inch to  $\frac{1}{4}$  of an inch.

It is desirable to remove nearly all the solvent remaining in the fibers after cutting and to adjust the moisture content to that at which cellulose acetate staple is normally sold. Any one of a number of anti-static agents may be applied at this point (after drying) and preferably this is done by spraying a solution or an aqueous emulsion of the desired anti-static agent onto the staple. Any of the following well known anti-static materials may be used for this purpose: diethyl cyclohexylamine salt of a long chain sulfate, cetyl betaine, lorolamine hydrochloride, salts of triethanolamine, reaction products of long chain amides and dimethyl sulfate, and sodium potassium ethyl phosphate.

I have found that only when the filament bundles are crinkled directly from the spinning machine or when the solvent content is appreciable (as well as an appreciable moisture content) that a satisfactory tow for direct conversion can be produced. However, other factors are also essential to produce a satisfactory tow for this purpose. As indicated above, a relatively deep coarse crinkle should be impressed in the filaments in order that the fibers formed therefrom will have adequate fiber adhesion in the spinning operation, for without sufficient and proper crinkle 5, 8 and 12 denier fibers cannot be handled in drawing operations.

When the tow of continuous crinkled filaments is to be shipped to a distant plant for conversion into top, it is desirable to wind the same into some sort of package from which it may be easily unwound. However, the winding of the crinkled tow while it contains in the neighborhood of 25 or 30% moisture plus solvent and storing such

packages for a period of time greatly reduces the intensity and uniformity of crinkle, due to differences in exposure and tension and/or pressure making the tow unsatisfactory for subsequent processing. On the other hand, when the tow of crinkled filaments is collected in loose coils, for instance in a perforated basket, and uniformly dried to reduce the moisture content to 6.0% or less and to substantially completely eliminate the solvent, it may be wound at relatively low tension onto tubes to form relatively large cylindrical packages (12 pounds or more) and even though stored for several months the crimp will be sufficiently retained for satisfactory processing. It is best to apply a finish at the spinning machine 15 free from any anti-static agent, for in subsequent cutting operations, the electrostatic charges on the filaments cause the cut fibers to strongly repel each other with the tendency for bundles of filaments to separate. The tow may vary widely 20 in size, for example, from 20,000 denier or less to 100,000 denier or more, although a tow of from 30,000 denier to 50,000 denier is generally preferred for practical reasons.

Whether the tow of crinkled filaments is to be cut as earlier described or converted by cutting the filaments without losing their parallelism and directly form therefrom a top, it is to be noted that during cutting a small but positive pull is needed to effectively separate the filaments and prevent "bundles." Because the tow of crinkled filaments after being subjected to tension is comprised largely of individual and separated filaments, when subjected to cutting, there is much greater resistance to fusing even though severed by scissors or other coating blade cutters. This improved resistance to fusing greatly widens the field of utility of this tow as compared with prior art tows of dry cellulose acetate filaments, for heretofore it has been considered essential to cut 40 dry cellulose acetate filaments with a single non-coating blade to prevent fusing and sticking together of the cut fiber ends.

By following this invention an extremely well-opened, essentially untangled, controlled crinkled cellulose acetate staple fiber of good strength that is eminently suited for handling on the cotton, woolen or worsted system to produce spun yarn of excellent quality may be produced. The tow

5 of crinkled filaments made and handled in accordance with this invention is extremely well suited for use in continuous processes for conversion of continuous filaments into staple and maintaining their substantial parallelism throughout the processing to produce a top or sliver. The very large bundle of filaments which can be crinkled or cut at one time and at a reasonably high rate of speed makes this process extremely economical to operate and because the filaments and fibers are maintained in an essentially dry condition (below approximately 40% solvent plus moisture), no expensive drying steps are needed as in the case where cellulose acetate fibers are crinkled by means of hot water or steam. More important than all the aforementioned advantages is the production of a uniformly high quality product which is easily and readily controlled according to the demands of the trade.

I claim:

The process which comprises forming a tow comprised of a plurality of cellulose acetate filaments of uniform denier within the range of 1.5 to 20 deniers, adjusting the moisture plus solvent content of said tow to within limits determined by the following formula, wherein  $d$  is the denier of the filaments:

Per cent moisture+solvent=40 log  $d-d+2\pm 6$   
30 the moisture plus solvent content in no case to be less than 8% or more than 40% by weight based on the weight of the dry cellulose acetate filaments, imparting to said tow by mechanical means a uniform crinkle, said crinkle being substantially transverse to the longitudinal axis of the filaments, cutting the crinkled tow into staple of uniform length while maintaining said tow under a tension within the range of from 0.005 to 0.04 gram per denier, and at a moisture plus solvent content within the limits determined by the following formula, wherein  $d$  is the denier of the filaments:

Per cent moisture+solvent=40 log  $d-d\pm 6$   
45 the moisture plus solvent content of the tow during cutting in no case to be less than 5% or more than 38% by weight based on the weight of the dry cellulose acetate filaments.

GILMAN STANLEY HOOPER.